

## UNITED STATES PATENT OFFICE.

ROBERT MEZGER, OF STUTTGART, GERMANY, ASSIGNOR TO THE FIRM: PAUL LECHLER,  
OF STUTTGART, GERMANY.

## METHOD OF COATING GASOMETERS.

No Drawing. Application filed July 10, 1925, Serial No. 42,841, and in Germany September 11, 1922.

My invention refers to an anti-corrosive adapted for use as a protective coating for gasometers and to the method of applying same.

5 As is well known to those skilled in the art the paint covering the gasometers is subjected to destruction by the water sealing the gasometer and by certain constituents dissolved in this water. It is further known 10 that this destructive action can be counteracted by covering the surface of the water seal with mineral oil having a high flash point. The gasometer, on being lowered into the water and on rising therein, will take 15 up some of the mineral oil which forms thereon a thin protective coating.

I have now ascertained that a solution of a bituminous substance in an oil which does not oxidize and which does not readily evaporate, for instance a solution of petroleum pitch in mineral oil, has superior protective properties which render a covering of paint unnecessary, whereby a great saving in material and expense is obtained.

25 I have found that a solution of at least 5 parts by weight of a neutral bituminous substance in not more than 95 parts by weight of an oil having a high flash point, being absolutely neutral and showing no 30 tendency to split off acids and gases, forms an excellent protection against the rusting of metals, allowing to obtain a permanent non-drying coating in consequence of the particular property of the bituminous substance of retaining the oil after the manner 35 of a sponge.

Thus while a thin film of said oil alone on the metal would gradually practically all run off, the bituminous substance acts to hold a thin film of the oil upon the vertical iron surface of the gasometer bell for a long 40 period of time.

Preferably about 20 parts of molten petroleum pitch are added with continuous stirring 80 parts mineral oil.

45 The gasometers are painted or sprayed with the protective solution both inside and outside. I may also cover the surface of the sealing water with a layer of the same solution. The protective solution forms a 50 fine mat coating on the gasometer which is automatically renewed when the gasometer is lowered into the water or raised therein, by contacting with the supernatant oil 55 solution.

This coating will never dry inasmuch as the bituminous substance retains the oil upon the iron surface after the manner of a sponge. The coating is therefore free to 60 adapt itself to all physical changes of the material so that there is no danger of the coating cracking and allowing moisture and air to attack the metal.

I wish it to be understood that I do not desire to be limited to the exact substances, 65 properties and operations above described, for obvious modifications will occur to a person skilled in the art.

I claim:—

70 The method of protecting bells of gasometers against corrosion, comprising applying to the surface to be protected a coating consisting of a solution of a neutral bituminous substance in an oil having a high flash point and which does not dry by oxidation, 75 and which is substantially non-volatile, and providing a body of the same solution in contact with the gas holder bell, whereby on being moved it will take up some of the solution.

80 In testimony whereof I affix my signature.

ROBERT MEZGER.